# EUROPEAN PATENT SPECIFICATION

(11) **EP 3 387 920 B1**
(45) Date of publication and mention of the grant of the patent: **29.12.2021**
(21) Application number: 16884894.3
(22) Date of filing: 13.01.2016
(51) Int. Cl.: A24C 5/56, D21H 13/08, D21H 13/14, D21H 15/02, D21H 19/10, D21H 19/20

(54) **TIPPING PAPER AND FILTERED CIGARETTE PRODUCT**
MUNDSTÜCKPAPIER UND GEFILTERTES ZIGARETTENPRODUKT
PAPIER MANCHETTE ET PRODUIT DE CIGARETTE À FILTRE

(43) Date of publication of application: 17.10.2018
(73) Proprietor: Japan Tobacco Inc., Tokyo 105-8422 (JP)
(72) Inventor: SAKURAI, Toru, Tokyo 130-8603 (JP)
(74) Representative: Hoffmann Eitle
(86) International application number: PCT/JP2016/050807
(87) International publication number: WO 2017/122291

(56) References cited:
- WO-A1-2007/074634
- WO-A1-2014/172192
- WO-A1-2015/108078
- JP-A- 2012 507 287
- JP-B2- 4 125 971
- JP-B2- 5 608 730
- US-A- 5 595 196

## Description

### Technical Field

This invention relates to a tipping paper and a filtered cigarette product.

### Background Art

A filtered cigarette product, for example, a filter-tipped cigarette is an article formed by placing a cigarette rod and filter in opposition to each other and in contact with each other, and winding a tipping paper around an outer circumferential surface of the filter and around an outer circumferential surface of the cigarette rod in the vicinity of the opposed part to thereby integrate the cigarette rod and filter into one article.

When a filter-tipped cigarette is smoked in a state where the smoker is wearing lipstick, the lipstick attached to the lip of the smoker adheres to the tipping paper, and the smoker has a feeling of discomfort in some cases for the reason that the lipstick comes off the lip to require fixing of the smoker's makeup, or that the lipstick adheres to the tipping paper to thereby spoil the external appearance of the cigarette, and so on.

In Patent Literature 1, a filter-tipped cigarette in which cigarette filter wrapping having a red color as a ground color is used, and which is thereby capable of making the lipstick adhering to the cigarette filter wrapping inconspicuous, and alleviating the feeling of discomfort of the smoker caused by the lipstick adhering to the cigarette filter wrapping to spoil the external appearance of the cigarette is disclosed.

In Patent Literature 2, a paper or nonwoven article comprises a nonwoven web layer. The nonwoven web layer comprises a plurality of fibers and a plurality of binder microfibers. The binder microfibers comprise a water non-dispersible, synthetic polymer. The binder microfibers have a length of less than 25 millimeters and a fineness of less than 0.5 d/f. The binder microfibers further have a melting temperature that is less than the melting temperature of the fibers. The nonwoven web layer may comprise a coating. After the nonwoven web layer is subjected to drying and thermal bonding, the coating may be applied to the nonwoven web and/or paper. The coating can comprise a decorative coating, a printing ink, a barrier coating, an adhesive coating, and a heat seal coating. The coating can comprise a liquid barrier and/or a microbial barrier.

In Patent Literature 3 a method for producing a filter cigarette with tipping paper having improved lip release properties is disclosed. Lip release chemicals are applied to one side of a base tipping paper during its manufacture in a papermaking process by surface coating, followed by manufacture of the cigarette using otherwise conventional apparatus and materials according to known procedures

### Citation List

### Patent Literature

Patent Literature 1: JP H10-136962 A
Patent Literature 2: WO 2014/172192 A1
Patent Literature 3: US 5,595,196 A

### Summary of Invention

### Technical Problem

However, the cigarette filter wrapping disclosed in Patent Literature 1 is not to prevent the adhering itself of the lipstick to the cigarette filter wrapping.

This invention relates to provide a tipping paper and a filtered cigarette product capable of reducing adhesion of lipstick to a tipping paper surface when the filtered cigarette product is smoked.

### Means for Solving the Problem

According to the present invention, a tipping paper characterized by including a front surface layer and back surface layer, and in which the front surface layer has surface properties satisfying a following formula (1) is provided. $- 8.2 \times Rsk - 0.2 \times Rc < 0$ (where Rsk is a skewness of the surface, and Rc is an average height)

The front surface layer (11) is a nonwoven fabric, and the nonwoven fabric is formed of wood pulp and rayon fiber with binder fiber, or of rayon fiber and binder fiber, wherein a fiber thickness is greater than or equal to 0.8dtex and less than or equal to 11dtex, the nonwoven fabric possesses a basis weight of greater than or equal to 10gsm and less than or equal to 70gsm, and the amount of the rayon fiber based on the total amount of the wood pulp and the rayon fiber with the binder fiber is greater than or equal to 40% by weight and less than or equal to 80% by weight.

### Advantageous Effects of Invention

The present invention can reduce adhesion of lipstick or the like to a tipping paper surface when a filtered cigarette product is smoked.

### Brief Description of Drawings

FIG. 1 is a schematic cross-sectional view of a tipping paper according to a first embodiment.
FIG. 2 is a schematic enlarged view of a nonwoven fabric.
FIG. 3 is a schematic cross-sectional view of a tipping paper according to a second embodiment.
FIG. 4 is a schematic cross-sectional view of a tipping paper according to a third embodiment.
FIG. 5 shows a tipping paper according to a fourth embodiment and, (A) is a perspective view of a back surface layer provided with a decorative section at an upper surface thereof, and (B) is a perspective view of the whole tipping paper.
FIG. 6 is a schematic cross-sectional view along a line VI-VI of FIG. 5.
FIG. 7 is a schematic cross-sectional view of a tipping paper according to a fifth embodiment.
FIG. 8 is a schematic cross-sectional view of a tipping paper according to a sixth embodiment.
FIG. 9 is a schematic cross-sectional view of a tipping paper according to a seventh embodiment.
FIG. 10 is a perspective view showing a filtered cigarette according to an eighth embodiment.
FIG. 11 is a view for explaining a method of attaching lipstick to tipping paper by using a rheometer.
FIG. 12 is a view showing a relationship between the surface roughness and color difference ΔE.
FIG. 13 is a view showing a result of a sensory evaluation.

Mode for Carrying Out the Invention Hereinafter, several embodiments will be described with reference to the accompanying drawings. Elements common throughout the embodiments are to be denoted by identical reference symbols, and duplicated explanation is omitted. Further, each drawing is a schematic view for promoting understanding of the embodiment, and there are positions different from the actual situation in shape, dimensions, and ratio. Further, in this specification, in order to indicate a relative positional relationship, although terms "above", "below", and the like are appropriately used in correlation with the drawings, these terms are not to specify the absolute positional relationship.

### (First Embodiment)

FIG. 1 is a schematic cross-sectional view of a tipping paper 1 according to a first embodiment. The tipping paper 1 is provided with a front surface layer 11 and a back surface layer 12.

The front surface layer 11 has surface properties which satisfy a formula (1): -8.2×Rsk-0.2×Rc<0. In the formula (1), Rsk represents the skewness, and Rc represents the average height. The tipping paper has the surface properties indicated by the formula (1), whereby it is possible to reduce the area of contact between the lip and tipping paper. It is more desirable that the front surface layer 11 should have surface properties which satisfy a formula (2): -8.2×Rsk-0.2×Rc<-20. The surface properties indicated by the formulae (1) and (2) will be described later.

The front surface layer 11 is normally formed of a material producing surface properties specified by the above formula (1) with respect to the upper surface profile (concavo-convex shape) thereof. Examples of such a material include an aggregate of partially combined fibers, for example, a nonwoven fabric. In FIG. 2, a part of the flat surface of such a nonwoven fabric is shown in an enlarging manner. A plurality of fibers (fibers for nonwoven fabric) 13 constituting the nonwoven fabric are combined with each other at combining parts 14 through fusion bonding substances 15 to thereby form an aggregate. The fiber 13 is a rayon fiber. The fusion bonding substance 15 is a substance formed when a binder fiber such as a polyvinyl alcohol (PVA) fiber, polyethylene glycol (PEG) fiber, vinylon fiber is melted in the process of putting the front surface layer 11 and back surface layer 12 one on top of the other to dry the layers 11 and 12 to be described later, and combines the fibers 13 for the nonwoven fabric with each other. The nonwoven fabric may include pulp in addition to the fibers 13 for the nonwoven fabric and binder fiber. In the nonwoven fabric, each of constituent fibers has a thickness greater than or equal to 0.8dtex and less than or equal to 11dtex, and has a basis weight greater than or equal to 10 and less than or equal to 70gsm. In a preferred embodiment, in a nonwoven fabric, each of constituent fibers has a thickness greater than or equal to 3.3dtex and less than or equal to 11dtex, and has a basis weight greater than or equal to 10gsm and less than or equal to 70gsm. Further, the nonwoven fabric may be colored by a dye such as a food additive colorant or the like. It should be noted that in this specification, the "nonwoven fabric" includes paper. In general, as a method of forming a nonwoven fabric, for example, a dry method, a wet method, a spunbonding method, a melt-blowing method, and an air-laid method are known. Further, as a method of combining fibers constituting the nonwoven fabric with each other, for example, a chemical bonding method, a thermal bonding method, a needle punching method, and a hydroentangling method are known. Although the nonwoven fabric contained in the front surface layer 11 is formed by the wet method, and fibers 13 for the nonwoven fabric are combined with each other by the thermal bonding method, as the method of forming the nonwoven fabric and the method of combining the nonwoven fabric fibers 13, other generally known methods may also be used.

In Table 1, general physical properties required of the tipping paper are shown. In order that the tipping paper 1 can satisfy, as a whole, the general physical properties required of the tipping paper, for example, tensile strength or the like, a back surface layer 12 can be provided on the under surface of the front surface layer 11. The back surface layer 12 can be formed of a material known in the field concerned as a material for the tipping paper, for example, pulp or the like.

**Table 1**

| Physical Properties | Units | Range |
|---|---|---|
| Tensile Strength | N/15mm | 26.0≤ |
| Elongation | % | 1.4≤ |

The tipping paper 1 can be obtained by combining the front surface layer 11 and back surface layer 12 with each other by a papermaking method well known to those skilled in the art. This papermaking method includes at least a process of combining a material constituting the front surface layer 11 and material constituting the back surface layer 12 with each other, and a process of drying the resultant. As the paper machine, conventionally known ones, for example, a cylinder paper machine, inclined tanmo machine, fourdrinier paper machine, tanmo machine, and the like can be used, and paper machines can be appropriately combined according to the prescribed properties. This papermaking method includes, for example, a process of combining wet paper formed of a suspension of a material constituting the front surface layer 11 by means of a cylinder paper machine and wet paper formed of a suspension of a material constituting the back surface layer 12 by means of a fourdrinier paper machine with each other. Further, the wet paper combined in this way can be dried by using conventionally known drying methods such as the yankee dryer method, multi-cylinder method, hot-air method, infrared heating method, and the like. In one embodiment, the wet paper laminated body of the front surface layer 11 and back surface layer 12 can be dried by using a dryer of a temperature of 100°C to 150°C.

It should be noted that at this time, fibers contained in the front surface layer 11 and having adhesiveness when melted, such as polyvinyl alcohol (PVA) fibers, polyethylene glycol (PEG) fibers, vinylon fibers are melted, whereby the fibers become fusion bonding substances 15 having adhesiveness and the fusion bonding substances 15 can combine fibers 13 constituting the front surface layer 11 with each other. It should be noted that regarding the method of combining the front surface layer 11 and back surface layer 12 with each other, the method is not limited to the aforementioned papermaking methods, and other conventionally known papermaking methods may also be used. As such papermaking methods, methods described in "Hand book of pulp and paper technology 1982", Japan Technical Association of the Pulp and Paper Industry, pp. 284 to 305 can be used.

The conventional tipping paper has, like the generally used printing paper, not a structure formed by combining two layers having different physical properties, and has a single layer structure, in which the surface properties of the front surface and back surface are approximately identical and the smoothness of both the surfaces is high. For this reason, in a filter-tipped cigarette provided with the conventional tipping paper, the tipping paper tends to come into close contact with the lip of the smoker at the time of smoking. As a result, lipstick or the like attached to the lip of the smoker becomes liable to move onto the tipping paper. Further, in the conventional tipping paper, there is sometimes a case where the lip is released from the tipping paper during smoking, the smoker's lip adheres to the tipping paper depending on the state of the smoker's lip or the environment and, when the adhesion is strong, there is even a case where the skin of the lip comes off.

However, the tipping paper 1 according to this embodiment is provided with the front surface layer 11 having surface properties satisfying the above formula (1), and thereby can reduce the area of contact between the lip and tipping paper 1, and hence can reduce adhesion of a substance such as lipstick attached to the surface of the smoker's lip to the tipping paper 1. Furthermore, even when lipstick is not used, it is possible to prevent unpleasant phenomena such as adhesion of the skin of the smoker's lip to the tipping paper, coming off of the skin of the lip when the lip is released from the tipping paper, and so on from occurring. The quality of the tipping paper which makes it easy for the tipping paper and lip to separate from each other when the cigarette is to be released from the lip is expressed by that the lip-releasability is excellent.

### (Second Embodiment)

In FIG. 3, a schematic cross-sectional view of a tipping paper 2 according to a second embodiment is shown. The tipping paper 2 according to the second embodiment has a configuration identical to the tipping paper 1 according to the first embodiment except that the front surface layer 11 and back surface layer 12 are stuck with an adhesive layer 21.

As the adhesive layer 21, a water-based adhesive or hot-melt adhesive can be used. As the water-based adhesive, for example, a starch-based, cellulose-based, PVA-based, polyvinyl acetate (PVAc)-based, and ethylene-vinyl acetate (EVA)-based adhesive can be used. As the hot-melt adhesive, a resin-based, polyethylene (PE)-based, and polypropylene (PP)-based adhesive can be used. When the resin-based adhesive is used as the adhesive, the resin-based adhesive layer 21 has a luster and reflects light incident on the resin-based adhesive layer 21, and hence it is possible to provide elegant tipping paper in which light leaks out of gaps between fibers of the front surface layer 11 to thereby impart a unique feeling to the tipping paper. Further, as the adhesive layer 21, a colored resultant formed by mixing the aforementioned adhesive with dye may also be used.

### (Third Embodiment)

In FIG. 4, a schematic cross-sectional view of a tipping paper according to a third embodiment is shown. The tipping paper according to the third embodiment has a configuration identical to the tipping paper 1 according to the first embodiment except that a coating agent layer 31 is provided on the upper surface of the front surface layer 11.

The coating agent layer 31 can be provided by applying a coating agent to the upper surface of the front surface layer 11. By providing the coating agent layer 31, it is possible to prevent fibers in the front surface layer 11 from falling off. As the coating agent, for example, starch, nitrocellulose or polyvinyl alcohol or a combination of these can be used. It is desirable that the coating agent be such an amount as not to significantly change the surface properties of the front surface layer 11. For example, it is desirable that the coating agent be less than or equal to 0.8gsm from the viewpoint of guaranteeing the surface properties of the nonwoven fabric.

### (Fourth Embodiment)

Next, a tipping paper 4 according to a fourth embodiment will be described below with reference to FIG. 5 and FIG. 6.

FIG. 5 shows the tipping paper 4 according to the fourth embodiment, and (A) is a perspective view of a back surface layer 12 of that, and (B) is a perspective view of the whole tipping paper 4. FIG. 6 is a schematic cross-sectional view along a line VI-VI of FIG. 5. The tipping paper 4 according to the fourth embodiment is provided with a front surface layer 11, back surface layer 12, and adhesive layer 21. As shown in FIG. 5(A), the back surface layer 12 is provided with a decorative section 41 on an upper surface (surface opposed to the front surface layer 11) thereof. The decorative section 41 can be provided by printing a decorative pattern on the upper surface of the back surface layer 12. Although the tipping paper 4 has a configuration identical to the tipping paper 2 according to the second embodiment except that the tipping paper 4 is provided with the decorative section 41 on the back surface layer 12, it is desirable that the adhesive to be used as the adhesive layer 21 (FIG. 6) be transparent so that the decorative section 41 can be seen through from the front surface layer 11 side.

As shown in FIG. 5(B), in the tipping paper 4, the decorative section 41 is provided on the upper surface of the back surface layer 12, whereby the decorative section 41 can be seen through from the front surface layer 11, thereby making the tipping paper 4 excellent in design.

### (Fifth Embodiment)

In FIG. 7, a schematic cross-sectional view of a tipping paper 5 according to a fifth embodiment is shown. The tipping paper 5 according to the fifth embodiment has a configuration identical to the tipping paper 1 according to the first embodiment except that a surface modifier layer 51 is provided on the upper surface of the front surface layer 11.

The surface modifier layer 51 can be provided by applying a surface modifier configured to prevent, for example, lipstick or the like from adhering to the tipping paper to the upper surface of the front surface layer 11. As the surface modifier, for example, a fluorine-based resin or silicon-based resin can be used. By forming the surface modifier layer 51, it is possible to further prevent substances from adhering to the surface of the tipping paper 5. The thickness of the surface modifier layer 51 can appropriately be adjusted according to the substance to be used as the surface modifier and the lipstick adhesion reducing effect required of the tipping paper 5.

### (Sixth Embodiment)

In FIG. 8, a schematic cross-sectional view of a tipping paper according to a sixth embodiment is shown. The tipping paper according to the sixth embodiment has a configuration identical to the tipping paper 1 according to the first embodiment except that an embossed pattern is provided on the front surface layer 11. The embossed pattern is constituted of a convex section 61 and concave section 62.

The embossed pattern can be provided by passing the tipping paper between a pair of embossing rolls.

By providing the embossed pattern on the front surface layer 11, it is possible to obtain a more lipstick adhesion reducing effect and, at the same time, provide tipping paper excellent in design. The embossing can be carried out to such a degree that the surface properties of the front surface layer 11 are not deteriorated.

### (Seventh Embodiment)

In FIG. 9, a schematic cross-sectional view of a tipping paper according to a seventh embodiment is shown. The tipping paper 7 according to the seventh embodiment has a configuration identical to the tipping paper 2 according to the second embodiment except that a front surface layer 11 is provided with, for example, a plurality of colored sections 71 separate from each other.

Each of the colored sections 71 extends from the upper surface of the front surface layer 11 to a plane thereof opposed to the back surface layer 12. The colored sections 71 can be formed by carrying out printing such as gravure printing, ink jet printing or the like using a colorant such as ink or the like. By providing the colored sections 71 in the front surface layer 11, it is possible to make a feeling different from a case where printing is carried out on normal tipping paper having a flat surface.

### (Eighth Embodiment)

Next, a filtered cigarette product according to an eighth embodiment will be described below. Here, although a filter-tipped cigarette will be described as an example of a filtered cigarette product, the filtered cigarette product is not limited to this and may be other smoking articles to which a filter is connected, such as a cigar and a cigarillo in addition to non-combustion smoking supplies and unheated smoking supplies, and the like which utilize electric heating/heat of chemical reaction.

As shown in FIG. 10, a filter-tipped cigarette 8 is provided with a cigarette rod 81, a filter 82 arranged in such a manner that an end part thereof is placed in opposition to and in contact with an end part of the cigarette rod 81, and a tipping paper 83 wound around the whole outer circumferential surface of the filter 82 and around the outer circumferential surface part of the cigarette rod 81 near the opposition/contact position, and integrating the cigarette rod 81 and filter 82 into one body. The cigarette rod 81 is provided with shredded tobacco 84 and rolled paper 85 wound around the shredded tobacco 84 into a cylindrical shape. The filter 82 is provided with a filter material (not shown) formed by binding or folding up, for example, acetate fibers or nonwoven fabric of pulp, and filter paper 86 rolling the filter material up into a cylindrical shape.

Such a filter-tipped cigarette 8 according to the embodiment can reduce adhesion of lipstick on the surface of the lip of the smoker to the tipping paper, while maintaining the functional characteristics (tensile strength and opacity) caused by the advantageous effects of the tipping paper according to each of the first to seventh embodiments.

### (Example)

In order to clarify a relationship between the surface properties of the tipping paper and lipstick adhering state, test samples were used to carry out (1) measurement of the lipstick adhering state and (2) sensory evaluation. Hereinafter, descriptions will be given in detail with reference to the accompanying drawings.

First, test samples different from each other in characteristics were prepared. Each of the test samples is provided with a front surface layer and a back surface layer. The front surface layer is constituted of a nonwoven fabric. The nonwoven fabric is formed of wood pulp and rayon fiber with binder fiber, or rayon fiber and binder fiber by hand making, and has different surface roughness, fiber length, and basis weight for each test samples. As the rayon fiber, that having a thickness of 0.1dtex to 11.0dtex was used. Further, test samples in which polyvinyl alcohol or starch was used as a coating agent for prevention of fiber falling-off were also manufactured.

As the back surface layer, paper formed by using wood pulp generally used as a material for tipping paper was used. Further, test samples in which the front surface layer and back surface layer were stuck with a vinyl acetate-based adhesive or resin-based adhesive were also manufactured.

It should be noted that measurement of the surface roughness was carried out by using SURFTEST SJ-210 (trade name) manufactured by Mitutoyo Corporation. The filtering process in the surface roughness measurement was carried out by using the Gaussian filter. Further, as the detector, that having a shape of a stylus front R of 2pm and front edge angle of 60° was used. The measurement condition was obtained by setting the standard condition in conformity with ISO1997 and setting the roughness curve R to cutoff values λc=2.5mm, λs=8µm, and number of sections (N) 4.

### (1) measurement of adhering state

### Reproduction of adhesion to lipstick

Adhesion of lipstick attached to the lip of a smoker to the tipping paper of a case where a filter-tipped cigarette is actually used was reproduced by using a rheometer. FIG. 11 is a view for explaining the method of making lipstick 95 adheres to the tipping paper 93 by using a rheometer (CR-3000EX-S manufactured by Sun Scientific Co., Ltd.).

FIG. 11(A) is a schematic view showing a state where tipping paper 93 of a test sample is put on the rheometer.

The rheometer is provided with a cylindrical plunger 91 having a diameter of 10mm, and measuring table 92 on which the tipping paper 93 of the test sample is to be placed. Next, the tipping paper 93 of the test sample is placed on the top surface of the measuring table 92 of the rheometer. A gel 94 is placed on the top surface of the tipping paper 93. The gel 94 have elasticity and softness similar to a human lip, and "HITOHADA^{®} gel" (trade name), product number: H0-1, manufactured by EXSEAL Co., Ltd. having such physical properties that the pressure thereof at the time of deformation by 1mm is 0.53N±0.34 was used. To the lower surface of the gel 94, i.e., to the surface of the tipping paper 93 side, lipstick 95 is applied. As the lipstick 95, Max Factor Angelic Lip Brilliante (trade name, product number B542) was used. A flat plate 96 is placed on the top surface of the gel 94. The flat plate 96 can equalize the pressure to be applied to the tipping paper 93 when the plunger 91 is pressed in the vertical direction against the gel 94 and the flat surface of the tipping paper 93. The flat plate 96 is a flat plate formed of, for example, plastic. The tipping paper 93, gel 94, and flat plate 96 are held between the plunger 91 and measuring table 92.

FIG. 11(B) is a view showing a state where fixed pressure is applied to the flat plate 96, tipping paper 93 and gel 94 in the vertical direction for a constant time by thrusting the plunger 91 in a direction perpendicular to the planes of the flat plate 96, gel 94, and tipping paper 93. At this time, the pressure to be applied to the tipping paper 93 was set in such a manner that the pressure reaches the maximum pressure 2.5N after an elapse of about one second from the start of application of pressure, and becomes 0N after an elapse of about two seconds in order that the pressure can become approximately equal to the pressure to be applied to the tipping paper when the filter-tipped cigarette is actually smoked. Further, at this time, setting was made in such a manner that the moving speed of the plunger 91 in the direction toward the measuring table 92 becomes 70mm/min. Thereby, the lipstick 95 attached to the gel 94 is transferred to the tipping paper 93, and it is possible to reproduce adhesion of the lipstick 95 to the tipping paper 93 of a case where a filter-tipped cigarette including the tipping paper 93 of the test sample is actually used.

### Measurement of Degree of Lipstick Adhesion

Measurement of the degree of adhesion of the lipstick to the tipping paper was carried out, after the lipstick was adhered to the tipping paper by using the rheometer as described above, by measuring a color difference ΔE between a place on the tipping paper to which the lipstick was adhered and place to which the lipstick was not adhered. Measurement of the color difference ΔE was carried out by means of a spectrophotometer (manufactured by X-Rite Inc., product name: SpectroEye) by obtaining an average value of coordinates of the L^{∗}a^{∗}b^{∗} color coordinate system of the color difference display method specified by CIE, and calculating a color difference ΔE between the place on the tipping paper to which the lipstick was adhered and place to which the lipstick was not adhered. It should be noted that the condition of measurement by the spectrophotometer was made that the light source was D65, light source filter was not used, and viewing angle was set to 2°.

### Result

A measurement result obtained by the above procedures will be described. It should be noted that as a result of carrying out similar measurement with respect to existing white tipping paper having 37gsm as a comparative example, a color difference ΔE of 51.2 was obtained.

First, relationships between the fiber length, fiber thickness, and color difference ΔE with respect to a test sample having a rayon combination ratio of 90% by weight, fibrous PVA combination ratio of 10% by weight, and basis weight of 30gsm are shown in Table 2. As is evident from Table 2, the larger the thickness of the fiber, the lower the color difference ΔE becomes, and it can be seen that it is desirable that the fibers of the nonwoven fabric be larger. Further, it was found that when the thickness of the fibers is 0.8dtex or more, the color difference ΔE is lower than the color difference ΔE of the comparative example by about 10, and a lipstick adhesion reducing effect can be obtained. Furthermore, it was found that when the thickness of the fibers is 3.3dtex or more, the color difference ΔE is lower than the color difference ΔE of the comparative example by about 30 or more, and a more lipstick adhesion reducing effect can be obtained.

**Table 2**

| | Fiber Thickness (dtx) | Fiber Length (mm) | Color difference ΔE |
|---|---|---|---|
| Test Sample 1 | 0.8 | 2 | 31 |
| Test Sample 2 | 0.8 | 4 | 43 |
| Test Sample 3 | 0.8 | 10 | 31 |
| Test Sample 4 | 1.7 | 5 | 31 |
| Test Sample 5 | 1.7 | 10 | 31 |
| Test Sample 6 | 1.7 | 15 | 22 |
| Test Sample 7 | 3.3 | 5 | 21 |
| Test Sample 8 | 3.3 | 10 | 18 |
| Test Sample 9 | 3.3 | 20 | 25 |
| Test Sample 10 | 7.8 | 8 | 10 |
| Test Sample 11 | 11 | 10 | 10 |

Further, relationships between the basis weight, rayon combination ratio of the nonwoven fabric, and color difference ΔE with respect to a test sample which has a fibrous PVA combination ratio of 10% by weight, rayon combination ratio as shown in Table 3, and in which the remaining combination ratio is constituted of wood pulp, and the thickness of rayon is 7.8dtex are shown in Table 3. First, when an observation of a relationship between the basis weight and color difference ΔE is made, the lower the basis weight, the lower the color difference ΔE becomes, and hence it can be seen that it is desirable that the basis weight be lower. However, although not shown in Table 3, in a nonwoven fabric having a basis weight less than 10gsm, the gel gets into gaps between fibers of the nonwoven fabric to reach the back surface layer, and thus a result that the lipstick adhesion reducing effect was remarkably impaired was obtained, and hence it was found that it is desirable that the basis weight of a nonwoven fabric be greater than or equal to 10gsm. Next, when an observation of a relationship between the rayon combination ratio of the nonwoven fabric and color difference ΔE is made, the higher the rayon combination ratio of the nonwoven fabric, the lower the color difference ΔE becomes, and thus it can be seen that the higher the rayon combination ratio of the nonwoven fabric, the higher the lipstick adhesion reducing effect becomes.

**Table 3**

| | Basis Weight (gsm) | Rayon combination ratio (%) | Color difference ΔE |
|---|---|---|---|
| Test Sample 12 | 30 | 40 | 21.6 |
| Test Sample 13 | 30 | 60 | 17.9 |
| Test Sample 14 | 30 | 80 | 11. 9 |
| Test Sample 15 | 50 | 40 | 31.0 |
| Test Sample 16 | 50 | 60 | 19.8 |
| Test Sample 17 | 50 | 80 | 12.4 |
| Test Sample 18 | 70 | 40 | 34.8 |
| Test Sample 19 | 70 | 60 | 21.7 |
| Test Sample 20 | 70 | 80 | 13.6 |

Further, the highest lipstick adhesion reducing effect was obtained by the tipping paper of the test sample which has a rayon combination ratio of 90% by weight, fibrous PVA combination ratio of 10% by weight, and basis weight of 15gsm, and in which a starch coating agent is used among the test samples.

Relationship between Surface roughness and Color difference

Further, data on the surface roughness and color difference ΔE obtained in the manner described above was used to carry out multiple regression analysis in which the color difference ΔE was used as an objective variable and various roughness parameters were used as dependent variables. As a result, regarding the roughness parameter, it was found that the color difference ΔE can be estimated by using two variables of the skewness Rsk and average height Rc. That is, it was found that the color difference ΔE is obtained from the skewness Rsk and average height Rc according to a formula: ΔE=-8.18×Rsk-0.21×Rc+40, and the condition of the lipstick adhering to the tipping paper can be estimated from the color difference ΔE. It should be noted that the square of the multiple correlation coefficient by the correlation analysis was r²=0.82. Further, the square (r²) of the single correlation coefficient by the single correlation analysis of each of the Rsk and Rc, r² was 0.28 in the Rsk, and r² was 0.67 in the Rc. When it is desired to lower the color difference ΔE, i.e., when it is desired to enhance the lipstick adhesion reducing effect, it is sufficient if the Rsk is increased in order to reduce the area of contact between the lip and tipping paper and/or it is sufficient if the Rc is increased in order to reduce the influence due to biting of the lip into gaps between fibers of the front surface layer.

FIG. 12 is a view formed by setting the skewness (Rsk) to the X-axis coordinate value, and average height (Rc) to the Y-axis coordinate value, and plotting measurement results of thirty-eight test samples, and is a view showing relationships between the surface roughness and color difference ΔE. It should be noted that in figure, in the measured color difference ΔE, a test sample with ΔE<10 is indicated by a white circular plot, test samples with 10≤ΔE<20 are indicated by black circular plots, test samples with 20≤ΔE<30 are indicated by white square plots, and test samples with 30≤ΔE<40 are indicated by black square plots, respectively. Further, a measurement result of the case where existing white tipping paper having 37gsm was used as a comparative example is indicated by a white triangular plot.

Further, lines in figure express straight lines specified by a ΔE=-8.18×Rsk-0.21×Rc+40 and, respectively indicate a line (solid line) of a case where ΔE in the formula of straight lines is 10, line (alternate long and short dash line) of a case where ΔE is 20, line (broken line) of a case where ΔE is 30, and line (dotted line) of a case where ΔE is 40.

As described previously, the color difference ΔE measured with respect to the existing white tipping paper having 37gsm of the comparative example is 51.2. When assuming such a level that can be visually recognized in comparison with the color difference ΔE measured with respect to the existing white tipping paper having 37gsm of the comparative example to be a color difference ΔE=10 corresponding to one rate of the Munsell chroma, i.e., to be a level which can be recognized if the level is lower than the color difference ΔE measured with respect to the comparison example by 10 or more, all the color differences ΔE measured with respect to the tipping paper of the test samples plotted in FIG. 10 were less than 40, and were on the recognizable level.

Assuming that, on the basis of this result, a color difference ΔE<40 smaller than the color difference ΔE measured with respect to the existing white tipping paper having 37gsm by 10 or more is in the recognizable area, it is necessary that the formula (1): -8.2×Rsk-0.2×Rc<0 should be satisfied. Further, as a more remarkable effect, when a color difference ΔE<20 smaller than the color difference ΔE measured with respect to the existing white tipping paper having 37gsm by 30 or more is required, it is necessary that the formula (2): -8.2×Rsk-0.2×Rc<-20 should be satisfied.

As described above, it was found that a state of adhesion of a substance attached to the surface of a lip to the tipping paper can be calculated by parameterizing the state of adhesion by means of the surface properties (Rsk and Rc) of the front surface layer.

### (2) Sensory Evaluation

Filter-tipped cigarettes each provided with tipping paper of the test samples were actually used by six female panelists in a state where lipstick is attached to the lip or in a state where lipstick attached to the lip is once wiped off by means of tissue paper or the like, whereby sensory evaluation of the state of adhesion of the lipstick to the tipping paper was carried out. In FIG. 13, the results are shown. FIG. 13 is a view formed by plotting the evaluation results in a state where the horizontal axis is set to the measured color difference ΔE, and the longitudinal axis is set to the sensory amount. Evaluation results of the test samples are indicated by white rhombic plots, and evaluation results of the comparative example are indicated by black rhombic plots. It should be noted that regarding the sensory amount in the drawing, when it was felt by the female panelists that adhesion of lipstick to the tipping paper was not found at all, evaluation was made as a numerical value of "0", when it was felt that slight adhesion of lipstick was found, evaluation was made as "1", when it was felt that adhesion of lipstick was felt to a certain degree, evaluation was made as "2", when it was felt that adhesion of lipstick was evidently found, evaluation was made as "3", when it was felt that adhesion of lipstick was considerably found, evaluation was made as "4", and when it was felt that adhesion of lipstick was remarkably found, evaluation was made as a numerical value of "5", and the sensory amount is a value acquired by averaging the numerical values obtained from the six female panelists. Further, each of the quadrilaterals surrounding the plotted points in figure indicates a range of variation of 1σ. That is when the variation in the results of the answers is large, the quadrilateral becomes larger and, when the variation is small, the quadrilateral becomes smaller. Further, regarding the straight lines connecting plotted points and quadrilaterals indicating the ranges of variations in the test samples and comparative example, when evaluation of a case where the lipstick is not wiped off by using tissue paper or the like is to be indicated, the evaluation is indicated by a solid line and, when evaluation of a case where the lipstick is once wiped off is to be indicated, the evaluation is indicated by dotted lines.

As is evident from FIG. 13, in the sensory evaluation of the case where the lipstick attached to the lip is not wiped off by using tissue paper or the like, the comparative example was evaluated as "considerable adhesion" and, conversely, the test samples was evaluated as "a certain degree of adhesion", and the sensory amount associated with the state of adhesion of the lipstick to the tipping paper is lowered. Further, regarding the color difference ΔE, ΔE is also about 50 in the comparative example and, conversely, ΔE is measured about 30 in the test samples, and is lowered like the sensory amount and, it can be seen that when the lipstick attached to the lip is not wiped off by using tissue paper or the like, there is a correlation relationship between the color difference ΔE and sensory amount.

Further, in the sensory evaluation of the case where the lipstick attached to the lip is once wiped off by using tissue paper or the like, the comparative example was evaluated as "a certain degree of adhesion" and, conversely, the test samples was evaluated as "slight adhesion", and the sensory amount associated with the state of adhesion of the lipstick to the tipping paper is lowered. Further, regarding the color difference ΔE, ΔE is also about 20 in the comparative example and, conversely, ΔE is measured about 7 in the test samples, and is lowered like the sensory amount and, it can be seen that even when the lipstick attached to the lip is once wiped off by using tissue paper or the like, there is a correlation relationship between the color difference ΔE and sensory amount.

Further, when the lip-releasability of the test samples was measured in the similar manner, it was found that the test samples have lip-releasability overwhelmingly superior to the tipping paper of the comparative example.

Thus, when a questionnaire was carried out for the above six panelists about whether or not they are charmed by the test samples and tipping paper of the comparative example as a lipstick adhesion reducing product, all the members answered "not feel charm" in the comparative example and, conversely, in the tipping paper of the test samples, one panelist answered "greatly feel charm", one panelist answered "considerably feel charm", three panelists answered "feel a certain degree of charm", one panelist answered "slightly feel charm", and thus it was found that the tipping paper of the test samples is overwhelmingly improved in charm as compared with the existing white tipping paper of the comparative example having 37gsm.

As described above, it was demonstrated that the tipping paper of the test samples has a lipstick adhesion reducing effect and lip-releasability effective in the sensory evaluation.

### Reference Signs List

1 ··· tipping paper according to the first embodiment 11 ··· front surface layer 12··· back surface layer 13 ··· fiber 14 ··· combining part 15 ··· fusion bonding substances 2 ··· tipping paper according to the second embodiment 21 ··· adhesive layer 3 ··· tipping paper according to the third embodiment 31 ··· coating agent layer 4 ··· tipping paper according to the fourth embodiment 41 ··· decorative section 5 ··· tipping paper according to the fifth embodiment 51 ··· surface modifier layer 6 ··· tipping paper according to the sixth embodiment 61 ··· convex section 62 ··· concave section 7 ··· tipping paper according to the seventh embodiment 71 ··· colored section 8 ··· filter-tipped cigarette 81 ··· cigarette rod 82 ··· filter 83 ··· tipping paper 84 ··· shredded tobacco 85 ··· rolled paper 86 ··· filter paper 91 ··· plunger 92 ··· measuring table 93 ··· tipping paper 94 ··· gel 95 ··· lipstick 96 ··· flat plate

## Claims

1. A tipping paper (1) **characterized by** comprising:
a front surface layer (11) and a back surface layer (12), wherein
the front surface layer (11) possesses surface properties which satisfy a following formula (1): $- 8.2 \times Rsk - 0.2 \times Rc < 0 ,$
where Rsk is skewness of the surface, and Rc is an average height,
where Rsk and Rc are measured by using SURFTEST SJ-210 manufactured by Mitutoyo Corporation,
the front surface layer (11) is a nonwoven fabric, and
the nonwoven fabric is formed of wood pulp and rayon fiber with binder fiber, or of rayon fiber and binder fiber, wherein
a fiber thickness is greater than or equal to 0.8dtex and less than or equal to 11dtex,
the nonwoven fabric possesses a basis weight of greater than or equal to 10gsm and less than or equal to 70gsm, and
the amount of the rayon fiber based on the total amount of the wood pulp and the rayon fiber with the binder fiber is greater than or equal to 40% by weight and less than or equal to 80% by weight.

2. The tipping paper (1) according to Claim 1 **characterized in that** the front surface layer (11) possesses surface properties which satisfy a following formula (2). $- 8.2 \times Rsk - 0.2 \times Rc < - 20$

3. The tipping paper (1) according to Claim 1 or 2, **characterized in that** the front surface layer (11) includes an aggregate of partially combined fibers.

4. The tipping paper (1) according to Claim 1 to 3, **characterized in that** the nonwoven fabric is formed of wood pulp and rayon fiber, or rayon fiber with a thickness of greater than or equal to 3.3dtex and less than or equal to 11 dtex.

5. The tipping paper (1) according to any one of Claims 1 to 4, **characterized in that** the nonwoven fabric includes a coating agent constituted of a polymer.

6. The tipping paper (1) according to Claim 5, **characterized in that** the coating agent is constituted of starch, nitrocellulose or polyvinyl alcohol or a combination of these.

7. The tipping paper (1) according to any one of Claims 1 to 6, **characterized in that** the front surface layer (11) and the back surface layer (12) are stuck with a water-based adhesive or a hot-melt adhesive.

8. The tipping paper (1) according to any one of Claims 1 to 7, **characterized in that** a surface of the back surface layer (12) opposed to the front surface layer (11) is decorated.

9. The tipping paper (1) according to any one of Claims 1 to 8, **characterized in that** the front surface layer (11) possesses a surface modifier constituted of a fluorine-based resin or a silicon-based resin on a surface.

10. The tipping paper (1) according to any one of Claims 1 to 9, **characterized in that** the front surface layer (11) possesses an embossed pattern.

11. A filtered cigarette product (8) **characterized by** comprising: a cigarette rod (81); a filter (82); and a tipping paper (83) connecting the cigarette rod (81) and the filter (82), wherein the tipping paper (83) is the tipping paper (1) according to any one of Claims 1 to 10.

## Patentansprüche

1. Mundstückpapier (1), dadurch charakterisiert, dass es umfasst:
eine vorderseitige Oberflächenschicht (11) und eine rückseitige Oberflächenschicht (12), wobei die vorderseitige Oberflächenschicht (11) Oberflächeneigenschaften aufweist, die der folgenden Formel (1) genügen: $- 8,2 \times Rsk - 0,2 \times Rc < 0 ,$
wobei Rsk eine Schiefe der Oberfläche ist und Rc eine durchschnittliche Höhe ist,
wobei Rsk und Rc unter Verwendung von SURFTEST SJ-210, hergestellt von Mitutoyo Corporation, gemessen werden,
die vorderseitige Oberflächenschicht ein Vliesstoff ist, und
der Vliesstoff aus Zellstoff und Reyonfaser mit Bindefaser oder aus Reyonfaser und Bindefaser gebildet ist, wobei
eine Faserdicke größer als oder gleich 0,8 dtex und kleiner als oder gleich 11 dtex ist,
der Vliesstoff ein Flächengewicht von größer als oder gleich 10 gsm und kleiner als oder gleich 70 gsm aufweist, und
die Menge der Reyonfaser, bezogen auf die Gesamtmenge des Zellstoffs und der Reyonfaser mit der Bindefaser, größer als oder gleich 40 Gew.-% und kleiner als oder gleich 80 Gew.-% ist.

2. Mundstückpapier (1) gemäß Anspruch 1, dadurch charakterisiert, dass die vorderseitige Oberflächenschicht (11) Oberflächeneigenschaften aufweist, die der folgenden Formel (2) genügen. $- 8,2 \times Rsk - 0,2 \times Rc < - 20$

3. Mundstückpapier (1) gemäß Anspruch 1 oder 2, dadurch charakterisiert, dass die vorderseitige Oberflächenschicht (11) ein Aggregat aus partiell kombinierten Fasern enthält.

4. Mundstückpapier (1) gemäß Anspruch 1 bis 3, dadurch charakterisiert, dass der Vliesstoff aus Zellstoff und Reyonfaser oder Reyonfaser mit einer Dicke von größer als oder gleich 3,3 dtex und kleiner als oder gleich 11 dtex gebildet ist.

5. Mundstückpapier (1) gemäß einem der Ansprüche 1 bis 4, dadurch charakterisiert, dass der Vliesstoff ein Beschichtungsmittel, bestehend aus einem Polymer, enthält.

6. Mundstückpapier (1) gemäß Anspruch 5, dadurch charakterisiert, dass das Beschichtungsmittel aus Stärke, Nitrocellulose oder Polyvinylalkohol oder einer Kombination dieser besteht.

7. Mundstückpapier (1) gemäß einem der Ansprüche 1 bis 6, dadurch charakterisiert, dass die vorderseitige Oberflächenschicht (11) und die rückseitige Oberflächenschicht (12) mit einem wasserbasierten Klebstoff oder einem Schmelzklebstoff verklebt sind.

8. Mundstückpapier (1) gemäß einem der Ansprüche 1 bis 7, **dadurch gekennzeichnet, dass** eine Oberfläche der rückseitigen Oberflächenschicht (12), die der vorderseitigen Oberflächenschicht (11) gegenüberliegt, dekoriert ist.

9. Mundstückpapier (1) gemäß einem der Ansprüche 1 bis 8, dadurch charakterisiert, dass die vorderseitige Oberflächenschicht (11) auf einer Oberfläche einen Oberflächenmodifikator, bestehend aus einem fluorbasierten Harz oder einem silikonbasierten Harz, aufweist.

10. Mundstückpapier (1) gemäß einem der Ansprüche 1 bis 9, dadurch charakterisiert, dass die vorderseitige Oberflächenschicht (11) ein geprägtes Muster aufweist.

11. Gefiltertes Zigarettenprodukt (8), dadurch charakterisiert, dass es umfasst: eine Zigarettenstange (81); einen Filter (82); und ein Mundstückpapier (83), das die Zigarettenstange (81) und den Filter (82) verbindet, wobei das Mundstückpapier (83) das Mundstückpapier (1) gemäß einem der Ansprüche 1 bis 10 ist.

## Revendications

1. Papier de manchette (1) **caractérisé en ce qu'**il comprend :
une couche de surface avant (11) et une couche de surface arrière (12), dans lequel
la couche de surface avant (11) possède des propriétés de surface qui satisfont une formule (1) suivante : $- 8,2 \times Rsk - 0,2 \times Rc < 0 ,$
où Rsk est l'asymétrie de la surface, et Rc est une hauteur moyenne,
où Rsk et Rc sont mesurés en utilisant SURFTEST SJ-210 fabriqué par Mitutoyo Corporation,
la couche de surface avant (11) est un textile non tissé, et
le textile non tissé est formé de pâte de bois et fibre de rayonne avec fibre de liant, ou de fibre de rayonne et fibre de liant, dans lequel
une épaisseur de fibre est supérieure ou égale à 0,8 dtex et inférieure ou égale à 11 dtex,
le textile non tissé possède une masse de base supérieure ou égale à 10 g/m² et inférieure ou égale à 70 g/m², et
la quantité de la fibre de rayonne sur la base de la quantité totale de la pâte de bois et la fibre de rayonne avec la fibre de liant est supérieure ou égale à 40 % en masse et inférieure ou égale à 80 % en masse.

2. Papier de manchette (1) selon la revendication 1, **caractérisé en ce que** la couche de surface avant (11) possède des propriétés de surface qui satisfont une formule (2) suivante. $- 8,2 \times Rsk - 0,2 \times Rc < - 20$

3. Papier de manchette (1) selon la revendication 1 ou 2, **caractérisé en ce que** la couche de surface avant (11) inclut un agrégat de fibres partiellement combinées.

4. Papier de manchette (1) selon les revendications 1 à 3, **caractérisé en ce que** le textile non tissé est formé de pâte de bois et fibre de rayonne, ou fibre de rayonne avec une épaisseur supérieure ou égale à 3,3 dtex et inférieure ou égale à 11 dtex.

5. Papier de manchette (1) selon l'une quelconque des revendications 1 à 4, **caractérisé en ce que** le textile non tissé inclut un agent de revêtement constitué d'un polymère.

6. Papier de manchette (1) selon la revendication 5, **caractérisé en ce que** l'agent de revêtement est constitué d'amidon, nitrocellulose ou poly(alcool vinylique) ou une combinaison de ceux-ci.

7. Papier de manchette (1) selon l'une quelconque des revendications 1 à 6, **caractérisé en ce que** la couche de surface avant (11) et la couche de surface arrière (12) sont collées avec un adhésif à base d'eau ou un adhésif thermofusible.

8. Papier de manchette (1) selon l'une quelconque des revendications 1 à 7, **caractérisé en ce qu'**une surface de la couche de surface arrière (12) opposée à la couche de surface avant (11) est décorée.

9. Papier de manchette (1) selon l'une quelconque des revendications 1 à 8, **caractérisé en ce que** la couche de surface avant (11) possède un agent de modification de surface constitué d'une résine à base de fluor ou d'une résine à base de silicium sur une surface.

10. Papier de manchette (1) selon l'une quelconque des revendications 1 à 9, **caractérisé en ce que** la couche de surface avant (11) possède un motif bosselé.

11. Produit de cigarette à filtre (8) **caractérisé en ce qu'**il comprend : une tige de cigarette (81) ; un filtre (82) ; et un papier de manchette (83) raccordant la tige de cigarette (81) et le filtre (82), dans lequel le papier de manchette (83) est le papier de manchette (1) selon l'une quelconque des revendications 1 à 10.
